

Patented Feb. 5, 1929.

1,701,342

# UNITED STATES PATENT OFFICE.

FRANZ SKAUPY, OF BERLIN, GERMANY, ASSIGNOR TO GENERAL ELECTRIC COMPANY,  
A CORPORATION OF NEW YORK.

## FILAMENT FOR INCANDESCENT LAMPS AND THE LIKE.

No Drawing. Application filed April 20, 1925, Serial No. 24,674, and in Germany May 3, 1924.

The present invention relates to a process for improving the mechanical properties of crystalline nonmetallic substances used for filaments of incandescent lamps, space current devices, and the like.

It is an object of the invention to increase the tensile strength and plasticity of such substances.

Another object of the invention is to increase the size of the crystals as well as the limits of crystal growth of such substances.

The novel features which are believed to be characteristic of the invention are set forth with particularity in the appended 15 claims, the invention itself, however, both as to organization and method of operating together with further objects will best be understood by reference to the following specification.

20 In the manufacture of filaments for incandescent lamps vacuum tubes and the like it has been found desirable to transform the metallic conductor into one long continuous crystal. This is effected by methods well 25 known to the art involving the use of special molds, heat treatment, and gradual cooling.

Although applicable to metals such processes have been found unsuitable for the treatment of non-metallic substances which are 30 also suitable for filaments such as thorium oxide owing to the impossibility of working such substances into filamentary form without destruction.

35 In accordance with the present invention the difficulties associated with the working of such materials are obviated by surrounding them with metallic casings which may be removed at any desired stage of the working process, as hereinafter described.

40 In the preferred embodiment of the invention the difficultly fusible oxide, e. g. thorium oxide, is provided with such a casing by introducing the oxide in a pulverulent or molten state into a tube made of a suitable ductile metal, e. g. copper, nickel, or iron, although 45 more difficultly fusible metals such as tungsten may also be used. It is also possible to produce such a casing by electro-depositing the required metal upon the exterior of the

50 refractory oxide when the latter has been cast or agglomerated into a suitable coherent body. Another method of producing the casing is to electroplate the individual particles of the oxide with ductile metal and agglomer- 55 ate these into a coherent mass by means of

pressure while still another method of accomplishing the same result consists in producing a finely granular intimate mixture of the non-metallic substance, e. g. thorium oxide, with finely divided metal such as copper, 60 the mixture being so proportioned that the same will be sufficiently plastic for mechanical working at the temperatures chosen.

The oxide encased in the metal container produced as above described may now be 65 drawn down to any suitable size. The temperature at which the mechanical working is effected must be considerably above room temperature and not far removed from the melting point of the non-metallic substance since 70 it is well known that the plasticity thereof increases with a rise in temperature.

In order to induce the formation of a long continuous crystal in the oxide mass the entire structure may be subjected to a suitable 75 heat treatment which may for example consist in heating the structure to white heat or in moving the same through a plurality of zones of gradually increasing high temperature. The heating may also be induced by 80 passing a current of suitable strength through the non-metallic body. In order to improve the crystal structure obtained the rod or wire-shaped non-metallic body may be first preliminarily heated and then subjected to a 85 certain amount of tension so as to reduce it one or two stages whereupon it may again be reheated to a high degree.

This heat treatment which is intended to induce the formation of a single crystal may 90 be carried out either before or after the removal of the metal casing. The casing is removed preferably by dissolving the same in a suitable acid or by subjecting it to the action of a gas capable of attacking the metal, 95 such as hydrochloric acid gas. In the case of a metal of low fusing point the casing may even be removed by volatilization. When the filament has been produced by drawing down an agglomerated mixture of oxide and metal the metal may be so intimately associated with the oxide particles that the gaseous treatment above recited may be preferable for removing the metal.

The filament after the metal has been removed may be reduced further by drawing in order to close the pores resulting from the metal removal treatment and thus increase the solidity of the product.

The size of the crystals obtained and their 110

boundary limits will depend upon the nature and the degree of mechanical working to which the oxide is subjected as well as upon the temperature prevailing during the heat treatment and may also depend upon the preliminary condition of fineness of the material.

The crystal modification induced by the heat treatment is of especial advantage in 10 incandescent lamp and vacuum tube filaments since it is then possible to use the filaments without danger of recrystallization when subjected for a long time to high temperatures.

15 Under certain conditions it may also be preferable to change the oxide into a single crystal modification before subjecting it to mechanical working or drawing. Even in such a case, however, it is preferable to 20 close the non-metallic material in a ductile casing to protect the same from crumbling. By this means it is possible to draw the single crystal body out to a considerable extent and to convert it into the form of filamentary wire 25 suitable for use in electric lamps.

What I claim as new and desire to secure by Letters Patent of the United States, is:

1. The method for converting refractory oxides into a uni-crystal structure, comprising providing said material with a casing of 30 ductile metal, drawing to filamentary size,

passing a current through the drawn product of sufficient intensity to heat said product to convert it into a uni-crystal structure and removing said casing.

2. The method for converting non-crystalline oxides into a uni-crystal structure comprising placing said material within a tube of ductile metal, drawing to filamentary size, subjecting the drawn product to heat treatment to convert it into a uni-crystal structure and removing said tube.

3. The method for converting a non-crystalline oxide into a uni-crystal filament which comprises placing the oxide in a casing of 45 difficultly fusible metal, drawing the casing and enclosed oxide down to filamentary size and thereafter heat-treating the drawn filament to induce uni-crystal growth and removing the casing.

4. The method for converting a non-crystalline non-metallic filament into a uni-crystal, comprising encasing said filament within a casing of ductile metal, drawing the encased filament down to size, heat treating 50 said drawn filament to induce the growth of uni-crystal structure and removing said casing.

In witness whereof, I have hereunto set my hand this 3rd day of April, 1925.

FRANZ SKAUPY.